

1

3 663 436

**LUBRICATING GREASES**  
William D. Carswell, Chester, England, assignor to Shell  
Oil Co., New York, N.Y.

Oil Company, New York, N.Y.  
No Drawing. Filed June 27, 1968, Ser. No. 740,487  
Claims priority, application Great Britain, July 13, 1967,  
32,205/67

Int. Cl. C10m 3/26

U.S. CL. 252—28

## 6 Claims

#### ABSTRACT OF THE DISCLOSURE

Copper corrosion resistant greases are obtained by incorporating therein a minor amount of a 3-amino-1,2,4-triazole.

This invention relates to lubricating greases containing certain triazoles as metal deactivators. More specifically, this invention relates to a lubricating grease comprising a lubricating oil, a thickener, and a minor proportion of a 1,2,4-triazole.

A disadvantage of many greases when in contact with a metal surface containing copper for a period of time at normal or moderate temperatures, i.e., about 60°C., is that the grease turns green and stains the metal. This is particularly true with certain clay greases containing pre-made waterproofed clay powders as a thickener, especially when glycerol is incorporated therein as an anti-wear agent. Furthermore, at high temperatures, e.g., 100–120°C., the grease darkens thereby masking the greening and allowing appreciably more staining to occur on the metal.

It has now been found that the addition of certain 1,2,4-triazoles to greases considerably reduces the amount of greening and/or darkening of the grease thereby lessening the staining of metal surfaces at normal and elevated temperatures. Furthermore, the addition of 1,2,4-triazoles to greases having glycerol incorporated therein, such as clay greases prepared by the "wet" process and lithium greases, greatly reduces the staining of metals containing copper at elevated temperatures.

The 1,2,4-triazoles which are useful in this invention are preferably 3-amino-1,2,4-triazoles having the formula:



and tautomers thereof, wherein  $R_1$  is a member selected from the group consisting of hydrogen, alkyl, phenyl and alkyl substituted phenyl;  $R_2$  and  $R_3$  are members selected from the group consisting of hydrogen, acyl and aroyl, at least one of  $R_1$ ,  $R_2$  and  $R_3$  being hydrogen.  $R_4$  is hydrogen and depending upon the tautomeric form may be attached to any of the nitrogen atoms comprising the triazole ring. Thus, the formula recited above embraces, for example, not only 3-substituted- and 3,5-substituted-1,2,4-triazoles, for example 3-amino-1,2,4-triazole, i.e.



and 3-amino-5-heptyl-1,2,4-triazole, i.e.

2



but also acylated and aroylated-1,2,4-triazoles which may be:



wherein  $R_5$  is a member selected from the group consisting of alkyl and aryl.

Preferable triazoles are those in which  $R_1$ ,  $R_2$  and  $R_3$  are hydrogen atoms. Preferably, when  $R_1$ ,  $R_2$  and  $R_3$  are not all hydrogen atoms, the desired number of carbon atoms in the R groups is less than 30 and preferably less than 7.

The 3-amino-1,2,4-triazoles of this invention can be used in any desired proportion. Generally proportions of about 0.001-2% by weight are used and concentrations of from about 0.1 to 0.5% by weight based on the total composition are preferred.

The base oils of the grease can be either synthetic lubricating oils or mineral lubricating oils. Synthetic oils such as diesters, complex esters, polysiloxanes, and polyphenylethers may be used. It is, however, preferred to use a mineral lubricating oil.

The thickener can be either organic or inorganic thickeners. Among the organic thickeners are the soaps, such as the alkali and alkaline earth metal salts of fatty acids, e.g., lithium hydroxystearate. It is preferred, however, to use an inorganic thickener and more preferably an oleophilic clay, i.e., a clay that has been rendered waterproof by the addition of a surfactant thereto.

Suitable clays have a substantial base exchange capacity of normally at least 25 milliequivalents (meq.) per 100 grams, preferably between 25 and 100 meq. per 100 grams. Particularly useful are the montmorillonite clays, and in particular those referred to as bentonites. The magnesium bentonites sometimes referred to as hectorites are particularly useful.

The clay can be made oleophilic by absorption thereon or reaction thereon with organic ammonia bases or their salts. Preferably, the clay is made oleophilic by coating with a cationic surface-active agent. Preferred surface-active agents or waterproofants are amino amides formed between aliphatic saturated or unsaturated monocarboxylic acids having 10 to 22 carbon atoms and alkylene polyamines. The alkylene polyamines are usually the bottoms products remaining from the manufacture of ethylene diamine, i.e., diethylene triamine and tetraethylene pentamine.

These waterproofants may be used in the proportion of 35-125% w. based on the clay, and the clay may be present in the grease in the proportion of about 2.5 to 10% w. based on the total grease composition.

In addition to the 1,2,4-triazoles, other additives may be present in the grease, such as anti-wear agents, e.g.,

glycerol, castor oil, antioxidants, e.g., aromatic amines and anti-corrosion agents, e.g., alkaline metal nitrates and extreme pressure agents, e.g., lead naphthenates or metal sulfides.

The greases may be prepared by either a "wet" or "powdered" process.

Thus in the "wet" process, the clay can be dispersed in water to form a 1-5% w. clay dispersion from which the gangue may be separated by sedimentation or centrifuging. The waterproofant, optionally 4-12% w. basis clay, of a strong mineral acid such as phosphoric acid, and at least part of the mineral oil are then added while agitating. An oil layer containing the oleophilic clay then separates from the water. The free water is removed and the clay/oil layer is heated to evaporate substantially any remaining water. The components are subjected to a high rate of shear, either during water evaporation or subsequent thereto, and any remaining desired lubricating oil and any additives such as the 1,2,4-triazoles are added in this final stage (wet process).

Sometimes the preparation of the grease from a pre-formed waterproofed clay powder is preferred. The degangued aqueous clay dispersion containing from 1-5% w. of clay and having a base exchange capacity of between 25 and 100 meq. of exchangeable base per 100 grams of clay is mixed with 35-125% w. based on the clay of a waterproofant, optionally 4-12% w. basis clay, of a strong mineral acid such as phosphoric acid, and 500 to 5000% w. based on the clay of a water-immiscible relatively volatile inert organic liquid, e.g., a naphtha having a boiling range of 230-300° F. or a kerosine having a boiling range of 330-390° F. or their mixtures. There is formed a base consisting of the clay, waterproofant and a minor proportion of water associated with the organic liquid together with a phase consisting of a major proportion of water. The latter phase is removed and the remaining water and organic liquid are volatilized by heat. There is thus formed a pulverulent or crumbly oleophilic clay product. A proportion of a lubricating oil, preferably 50-200% w. based on clay may be mixed with the clay prior to evaporation of water and volatile liquid. The presence of the lubricating oil at this stage promotes the maintenance of high thickening power of the clay product. As the proportion of lubricating oil is increased dispersal of the product in any medium at a later stage (such as in oil for the formation of grease) becomes progressively easier.

Alternatively a preformed clay powder is obtained by heating a degangued clay dispersion in water at 80° C. and adding, while stirring, the waterproofant, optionally a strong mineral acid such as phosphoric acid, to facilitate the coating of the clay surface. Thereafter the composition may be (1) spray dried to a powder containing 1 to 4% water or (2) filtered and then dried by any convenient

method, e.g. tray dried or (3) a small proportion of a mineral lubricating oil is added to the composition which is then filtered and dried.

The clay product is mixed with a lubricating oil in order to prepare the grease. Preferably the mixture is sheared at normal or elevated temperatures, e.g., 80° C., and any additives, such as the 1,2,4-triazoles are normally added together with the lubricating oil (powder process).

Since the present triazoles are relatively insoluble in mineral oils they may be incorporated in the oils by means of solvents such as ethylene glycol, diethylene glycol, glycerol and water at normal or elevated temperatures (e.g., 80° C.) and at high concentrations (e.g., as a 50/50% w. solution). Although these concentrates are not soluble in mineral oil, they can be dispersed very finely so that the formation of coarse particles in the grease is prevented. In some cases the triazoles precipitated out of the solution on cooling. This, however, did not appear to reduce their effectiveness or produce coarse particles in the grease.

The invention is illustrated by the following data.

A hectorite clay-based grease containing the amino amide reaction product of a mixture of alkylene polyamines and fatty acids was prepared by both the "wet" and the "powder" process. All the greases contain at least 0.5% w. glycerol.

The triazoles were dissolved in a suitable solvent at 80° C. to obtain a concentrate, which was added to the grease before homogenization or to the finished grease.

The greases were then tested in a brass disc test as follows.

A brass disc 38 mm. in diameter was polished with carborundum powder and cleaned with cotton wool. A layer of grease 30 mm. in diameter and 1 mm. thick was spread on the disc and the disc then placed in an oven during a certain time at a certain temperature.

The greening of the grease at 60° C., the darkening of the grease at 100° C. and 120° C., and the staining of the discs were then noted as follows:

|    |          |               |
|----|----------|---------------|
| 40 | 0—none   | 3—moderate    |
|    | 1—trace  | 4—severe      |
|    | 2—slight | 5—very severe |

The results are given in the following table (the first figure represents greening at 60° C. or darkening at 100° C. and 120° C., the second figure staining; percentages are by weight; EG=ethylene glycol, DEG=diethylene glycol, G=glycerol).

The results indicate that overall the 1,2,4-triazoles are superior to the 1,2,3-triazoles and benzotriazoles especially at elevated temperatures of 100° C. and 120° C. Furthermore better results are obtained with the 3-amino 1,2,4-triazoles at all temperatures and at lower concentrations.

TABLE

| Additive                    | Solvent | Concentration<br>Additive in—1 | Powder process           |                    |                         | Wet process              |                          |
|-----------------------------|---------|--------------------------------|--------------------------|--------------------|-------------------------|--------------------------|--------------------------|
|                             |         |                                | Sol-<br>vent,<br>percent | Grease,<br>percent | 60° C.<br>(20<br>hours) | 100° C.<br>(24<br>hours) | 120° C.<br>(24<br>hours) |
| Benzotriazole-----          | EG      | 50                             | 0.3                      | 1-1                | -----                   | -----                    | -----                    |
|                             | DEG     | 50                             | 0.1                      | 4-2                | 3-4                     | 3-4                      | -----                    |
|                             | DEG     | 50                             | 0.3                      | 1-1                | 3-3                     | 4-4                      | 2-1                      |
|                             | G       | 50                             | 0.1                      | 3-2                | 3-5                     | 4-4                      | 3-2                      |
|                             | G       | 50                             | 0.3                      | 1-0                | 3-3                     | 4-4                      | 2-2                      |
| 5-methyl benzotriazole----- | EG      | 50                             | 0.3                      | 1-1                | -----                   | -----                    | -----                    |
|                             | DEG     | 50                             | 0.1                      | 3-2                | 3-4                     | 4-2                      | -----                    |
|                             | DEG     | 50                             | 0.3                      | 1-1                | 3-1                     | 4-1                      | -----                    |
|                             | G       | 50                             | 0.1                      | 3-2                | 3-1                     | 4-1                      | -----                    |
|                             | G       | 50                             | 0.3                      | 1-0                | 3-1                     | 4-2                      | -----                    |
| 5-lauryl benzotriazole----- | DEG     | 50                             | 0.1                      | 4-3                | 3-4                     | 4-4                      | -----                    |
|                             | DEG     | 50                             | 0.3                      | 1-1                | 3-0                     | 4-1                      | -----                    |

TABLE—Continued

| Additive                    | Solvent          | Concentration<br>Additive in—<br>Sol-<br>vent,<br>percent | Powder process          |                          |                          | Wet process              |                          |
|-----------------------------|------------------|-----------------------------------------------------------|-------------------------|--------------------------|--------------------------|--------------------------|--------------------------|
|                             |                  |                                                           | 60° C.<br>(20<br>hours) | 100° C.<br>(24<br>hours) | 120° C.<br>(24<br>hours) | 100° C.<br>(24<br>hours) | 120° C.<br>(24<br>hours) |
| 3-amino 1,2,4-triazole..... | ( <sup>1</sup> ) | 50                                                        | 0-1                     | 1-1                      | -----                    | -----                    | -----                    |
|                             | DEG              | 33                                                        | 0.05                    | 1-0                      | 2-1                      | 2-1                      | -----                    |
|                             | DEG              | 50                                                        | 0.1                     | 1-0                      | 2-1                      | 2-1                      | 0-0                      |
|                             | G                | 50                                                        | 0.05                    | 0-1                      | 2-2                      | 3-1                      | 3-3                      |
|                             | G                | 50                                                        | 0.1                     | 0-0                      | 1-1                      | 3-1                      | 1-2                      |
| 1,2,3-triazole.....         | G                | 33                                                        | 0.1                     | 1-2                      | 3-2                      | 4-4                      | -----                    |
|                             | G                | 33                                                        | 0.3                     | 0-0                      | 3-3                      | 4-4                      | -----                    |
| 1,2,4-triazole.....         | G                | 50                                                        | 0.1                     | 4-4                      | 3-3                      | 4-3                      | -----                    |
|                             | G                | 50                                                        | 0.3                     | 0-4                      | 1-2                      | 3-2                      | -----                    |
| None.....                   |                  |                                                           | 4-3                     | 4-5                      | 5-5                      | 4-4                      | 5-5                      |

<sup>1</sup> Water

I claim as my invention:

1. A grease composition comprising a lubricating oil gelled to grease consistency by a thickener selected from the group consisting of metal soaps and oleophilic clays and containing a copper corrosion-reducing amount of a 20 1,2,4-triazole of the formula



and tautomers thereof.

2. A grease composition according to claim 1 wherein 30 the thickener is an oleophilic clay.

3. A grease composition according to claim 2 wherein the triazole comprises from about 0.001 to about 2.0% w. of the grease composition.

4. A grease composition according to claim 3 wherein 35 the lubricating oil is a mineral oil.

5. A grease composition according to claim 2 wherein the clay is coated with an amino amide waterproofant formed by the reaction of C<sub>10</sub>—C<sub>22</sub> carboxylic acids and alkylene polyamines.

6. A grease composition according to claim 5 wherein the clay is a performed coated powder.

## References Cited

## UNITED STATES PATENTS

|           |         |                 |          |
|-----------|---------|-----------------|----------|
| 2,618,605 | 11/1952 | Schaeffer       | 252—390  |
| 3,382,087 | 5/1968  | Ostrowski       | 252—390  |
| 2,890,170 | 6/1959  | Ragborg         | 252—50   |
| 3,006,848 | 10/1961 | Caruso          | 252—28   |
| 3,050,463 | 8/1962  | Peterson        | 252—28   |
| 3,179,590 | 4/1965  | Loeffler et al. | 252—28   |
| 3,183,241 | 5/1965  | Oja             | 252—49.5 |

## FOREIGN PATENTS

|           |        |               |        |
|-----------|--------|---------------|--------|
| 1,041,334 | 9/1966 | Great Britain | 252—21 |
|-----------|--------|---------------|--------|

DANIEL E. WYMAN, Primary Examiner

I. VAUGHN, Assistant Examiner

U.S. Cl. X.R.

40 252—42.4, 50, 390